# EUROPEAN PATENT SPECIFICATION

(11) **EP 0 712 532 B1**
(45) Date of publication and mention of the grant of the patent: **02.05.1997**
(21) Application number: 95907498.0
(22) Date of filing: 05.08.1994
(51) Int. Cl.: H01F 1/055, H01F 1/059

(54) **SmFeTa alloy with 4-5 at% Ta addition and the process of its preperation**
SmFeTa Legierung mit 4-5 at% Ta Zusatz und dessen Herstellungsverfahren
alliage SmFeTa à adjonction de 4-5 at% Ta et le procédé de sa préperation

(30) Priority: 06.08.1993 SI 9300422
(43) Date of publication of application: 22.05.1996
(73) Proprietor: INSTITUT JOZEF STEFAN, SI-61000 Ljubljana (SI)
(72) Inventor: SAJE, Boris, 61000 Ljubljana (SI); KOBE, BESENICAR, SPOMENKA, 61000 Ljubljana (SI); EDWARDS PLATTS, Adrian, Birmingham B29 7JA (GB); HARRIS, Ivor, Rex, Birmingham B29 7JA (GB)
(74) Representative: Rackette, Karl, Dipl.-Phys. Dr.-Ing
(86) International application number: SI9400014
(87) International publication number: WO9504996

(56) References cited:
- EP-A- 0 344 018
- JP-A- 525 592
- PATENT ABSTRACTS OF JAPAN vol. 17, no. 315 (C-1071) 16 June 1993 & JP,A,05 025 592 (M.TOSHIHIKO) 2 February 1993
- JOURNAL OF ALLOYS AND COMPOUNDS, vol.185, 1992, AMSTERDAM NL pages 251 - 258 A.E.PLATTZ ET AL cited in the application
- JOURNAL OF MAGNETISM AND MAGNETIC MATERIALS, vol.114, no.1/2, August 1992, AMSTERDAM NL pages 138 - 144 BO-PING HU ET AL
- IEEE TRANSACTIONS ON MAGNETICS., vol.30, no.2, 2 March 1994, NEW YORK US pages 690 - 692 B.SAJE ET AL

## Description

The invention relates to the Sm₂Fe₁₇ alloy with Ta addition, and to the process for producing this alloy, which is suitable as the basic material for the preparation of permanent magnets based on nitrides of intermetallic compounds of rare earth and transition metals.

Nitrides of binary intermetallic compounds between rare earths, in the following text designated as RE, and transition metals, in the following text designated as TM, thus Sm₂Fe₁₇Nₓ, are new ferromagnetic materials, first discovered by Coey J. M. D. and Sun H., published in J. Mag. Magn. Mat. 87, (1990), L251 (1). The preparation of these materials is described in the European applications EP 369097, EP 453270, EP 538643, EP 493019 and Canadian applications CA 2040686, CA 2058283.

In JP-A-05 25 592 a rare earth magnet materials are described, having a composition of general formula R_{X}Fe_{(1-X-Y-Z)}M_{Y}C_{Z} and in which R₂Fe₁₇ type tetragonal crystal constitutes the main phase, where said R comprises rare earth metal which includes at least one of Sm, Ce, Nd and Pr, M comprises at least one of Ti, Zr, Hf, V, Nb, Ta, Cr, Mo, W, Mn, Nl, Pd, Cu, Ag, Zn, Mg, B, Al, Ga, In, Si ans Sn in defined ranges of quantities. The material obtained has to be heat treated at 1000°C for 12 hours because of component segregation.

Permanent magnets based on the Sm₂Fe₁₇N₃-x ternary interstitial phase with a rhombohedral Th₂Zn₁₇ - type structure are considered to be competitive with the well-known Nd-Fe-B based magnets. The intrinsic properties of Sm₂Fe₁₇N₃₋ₓ, where x is approximately 0.3, include a higher Curie temperature (Tc) for 100 to 200°C and anisotropy field (Ha), and a slightly lover magnetisation saturation (Ms). The compound where RE is Sm possesses these beneficial properties due to Sm, which is the only RE with a preferential vector of magnetisation in the direction of c -axis of the rhombohedral structure, which is the necessary condition for high magnetocrystal anisotropy. For comparison the magnetic properties of Nd₂Fe₁₄B and Sm₂Fe₁₇N_{X} are as follows:
- Nd₂Fe₁₄B:: T_{c} = 588 K,
Ms = 1.60 T,
Ha = **5 970 kA/m**
(BH)max = 509 kJ/m³
- Sm₂Fe₁₇Nₓ:: T_{c} = 749 K,
Ms = 1.55 T,
Ha = **11 150 kA/m**
(BH)max = 472 kJ/m³

Unfortunately, Sm₂Fe₁₇ binary phase which is used for production of the Sm₂Fe₁₇N₃₋ₓ interstitial temary compound through a gas-phase interstitial modification process, forms through a peritectic reaction between primary crystallised iron and Sm- rich liquid: L(liquid) + Fe -> Sm₂Fe₁₇. This always leads to considerable amounts of free iron (up to 25 %.) and some SmFe₂ or SmFe₃ Sm-rich phases in the as cast state. Free iron especially, unless removed by a subsequent isothermal homogenization treatment, reduces the coercivity of the Sm₂Fe₁₇ nitride produced when used for permanent magnets.

The usual methods for creating an alloy without soft magnetic phases are either high temperature-long term annealing of the samarium-rich cast alloy (five days at 1050°C) or through the phase modification with the addition of a third alloying element (from the group of transition metals). The phase relation can be influenced by the addition of the third element, which modifies the crystallization and prevents the primary crystallization of free iron and leads to a two phase structure consisting of Sm₂Fe₁₇ phase and one paramagnetic intermediate Laves phase. Up to the present, research work in this field was focused on the addition of the elements Ti and Nb as elements which influence the phase relations, and is published in the open literature Reinch B., Grieb B., Henig E. T., Petzow G., IEEE Trans. Magn., 28, (1992), 2832 and Platts A. E., Harris I. R., Coey J. M. D., J. Alloys Comp., (1992), 251

Of the other transition elements it was shown that Zr, Mo, Hf, V, Ti and Ta also form intermediate Laves phases of the AB₂ - type. There were no data published or patented on the influence of these elements on the phase relationships in the system Sm-Fe-TM.

The technical problem of the preparation of a cast alloy without the formation of unfavourable secondary phases can be partially solved by high temperature-long term annealing of the samarium-rich as -cast alloy, which is an expensive process, or by influencing the phase modification by the addition of Nb or Ti.

The purpose and the aim of the invention relates to the Sm Fe Ta alloy with 4-5 at% Ta addition and to the process for producing this alloy with the corresponding properties. The production of the alloy should be cheap and comparatively easy.

The technical problem of the preparation of the cast alloy without the formation of unfavourable secondary phases is solved in the invention by Ta addition and with the appropriate casting technique. Tantalum forms a Pauli paramagnetic TaFe2 intermediate hexagonal Laves phase with iron, as described in the patent claims.

By this invention the preparation of as -cast alloy which contains a minimal quantity of free iron and other ferromagnetic phases is enabled. The as -cast alloy is suitable for the nitrogenation procedure without any subsequent annealing process. As such, the nitrogenated alloy is suitable as a basic material for the preparation of a new generation of permanent magnets of Sm₂Fe₁₇Nₓ type.

The following example is meant to illustrate preffered embodiment of this invention.

The alloy which contains a minimum quantity of free iron and other ferromagnetic phases, which diminish the hard magnetic coercivity of Sm₂Fe₁₇ alloy, is produced. The amount of soft magnetic phases is low enough that for the preparation of Sm₂Fe₁₇ alloy suitable for the nitrogenation and production of Sm₂Fe₁₇Nₓ, high temperature annealing can be avoided.

By this invention the alloy with the composition Sm₂Fe₁₇₋ₓTaₓ is produced by arc melting in an inert atmosphere of Ar purified with Ti as a getter.

As -cast alloys were prepared by arc-melting of samples in a Ti purified Ar atmosphere using elemental Sm (99.99 %), Fe (99.99 %) and Ta (99.9%). The Ta addition is between 1 to 5 at.%. Excess Sm was added to the nominal composition of Sm₂Fe₁₇₋ₓTaₓ (10 to 30 wt.%) to counterbalance Sm evaporation loses during melting. First Fe and Ta are melted and Sm is added later. The samples are remelted four times to improve macro and micro homogeneity. In some cases three times is sufficient and sometimes the melt has to be remelted several times additionally.

Microstructural analysis shows phase compositional changes, which are dependent upon the increasing Ta content of the alloys of nominal composition Sm₂Fe₁₇₋ₓTaₓ. From Fig. 1, which shows the microstructure of the tantalum -free alloy, we can see the normal appearance of the as -cast state of the nominally stoichiometric Sm₂Fe₁₇ alloy. Dendrites of primary crystallised iron (black) are surrounded by peritecticaly formed Sm₂Fe₁₇ phase (grey) with some Sm -rich phase which was identified as SmFe₂ (white). The microstructural morphology is typical for the as -cast alloy of stoichiometric composition with dendrites of primary recrystallised iron, surrounded by peritecticaly formed Sm₂Fe₁₇ phase and partly with the Sm -rich phase, identified as SmFe₂ phase, detrimental for the magnetic properties and which can be removed by the known method of high temperature long term annealing.

Figure 2 shows the microstructure of the alloy with a nominal composition of 5 at.% of Ta. No iron dendrites are observed and the microstructure consists of a mixture of only Sm₂Fe₁₇ (grey) and Tafe₂ (white) phases.

Qualitative confirmation of the presence of the two phases Sm₂Fe₁₇ and TaFe₂ in the as -cast alloy were confirmed by thermomagnetic analysis of the samples, which is normally used for Curie temperature determination of the extant phases.

The difference between the tantalum -free alloy and 5 at% Ta material is evident from Figure 3, where normalised temperature curves are shown for a) Ta -free alloy, b) alloy with 5 at.% Ta and c) TaFe₂ alloy. For the Ta -free alloy three characteristic steps appeared on the M = f(T) curve, corresponding to the Curie temperatures of Sm₂Fe₁₇, SmFe₂ and Fe respectively. The thermomagnetic curve of the 5 % Ta material shows only one large step, consistent with the Curie temperature of the Sm₂Fe₁₇ phase. A thermomagnetic scan of the TaFe₂ phase shows the paramagnetic nature of the phase.

Fig. 4 shows thermomagnetic curves normalised to the Curie temperature of the Sm₂Fe₁₇ phase for the alloys with a) 1% Ta, b) 2% Ta and c) 4% Ta. Thermomagnetic analysis also shows the increase in the Curie temperature as a function of the Ta concentration in the Sm₂Fe₁₇ phase.

The invention relates to the preparation of the cast alloy with a minimum amount of free iron and/or other soft magnetic phases, which is suitable for further nitrogenation without high temperature long term annealing. The as -cast alloy is suitable for the preparation of the Sm₂Fe₁₇₋ₓTaₓN_{3-y} compound. The most important advantage of the invention is the cheaper preparation procedure of the alloy. Ta addition is a new solution to the problem of the appearance of soft ferromagnetic phases which deteriorate the hard magnetic properties of the alloy.

## Claims

1. An Sm-Fe-Ta containing alloy, suitable as the basic material for preparation of permanent magnets of Sm₂Fe₁₇N₃₋ₓ type,
*characterized by*
addition of 4 at.% to 5 at.% of elemental Ta to elemental Sm with the addition of excess of 10 to 30 wt. % and elemental Fe material, to obtain nominal Sm₂Fe₁₇₋ₓTaₓ composition, and being processed to result in the cast alloy containing two main phases Sm₂Fe₁₇ and TaFe₂, with minimal quantities of free iron and other ferromagnetic phases.

2. A process for producing the Sm-Fe-Ta containing alloy as claimed in Claim 1,
*characterized in that*
the said process comprises the steps of allowing Fe and Ta after which Sm is added with an excess of 10 to 30 wt.% of nominal Sm₂Fe₁₇₋ₓTaₓ composition to compensate evaporation losses the addition of Ta being between 4 and 5 at% and that this Sm-Fe-Ta alloy is at least remelted three times, where said melting is arc-melting in a Ti purified Ar atmosphere.

## Patentansprüche

1. Sm-Fe-Ta enthaltende Legierung, die als Basismaterial zur Herstellung von Permanentmagneten des Typs Sm₂Fe₁₇N₃₋ₓ geeignet ist, **gekennzeichnet durch** den Zusatz von 4 at.% bis 5 at.% von elementarem Ta zu elementarem Sm mit dem Zusatz im Überschuß mit 10 bis 30 Gewicht% und elementares Fe-Material zum Erhalt einer Nennzusammensetzung Sm₂Fe₁₇₋ₓTaₓ und einer Verarbeitung zum Erhalt einer Gußlegierung mit zwei Hauptphasen Sm₂Fe₁₇ und TaFe₂ mit minimalen Mengen von freiem Eisen und anderen ferromagnetischen Phasen.

2. Verfahren zur Herstellung einer Sm-Fe-Ta enthaltenden Legierung nach Anspruch 1, **dadurch gekennzeichnet,** daß der Prozeß die Schritte des Legierens von Fe und Ta nach Zusatz von Sm im Überschuß mit 10 bis 30 Gewicht% zu einer Nennzusammensetzung Sm₂Fe₁₇₋ₓTaₓ zum Kompensieren von Verdampfungsverlusten und den Zusatz von Ta zwischen 4 und 5 at.% aufweist und daß diese Sm-Fe-Ta-Legierung wenigstens dreimal umgeschmolzen wird, wobei das Schmelzen ein Bogenschmelzen in einer Ti-gereinigten Ar-Atmosphäre ist.

## Revendications

1. Alliage contenant Sm-Fe-Ta convenable comme matériau de base pour la préparation d'aimants permanents de type Sm₂Fe₁₇₋ₓN₃₋ₓ,
*caractérisé* par l'addition de 4 at% à 5 at% de Ta élémentaire à du Sm élémentaire introduit en un excès de 10 jusqu'à 30% en poids et du Fe élémentaire, pour obtenir une composition nominale Sm₂Fe₁₇₋ₓTaₓ et qui est traitée pour fournir l'alliage coulé contenant deux phases principales Sm₂Fe₁₇ et TaFe₂, avec des quantités minimales de fer libre et d'autres phases ferromagnétiques.

2. Procédé pour la production de l'alliage contenant Sm-Fe-Ta suivant la revendication 1,
*caractérisé en ce que* ce procédé comprend les étapes d'alliage de Fe et de Ta, après quoi du Sm est ajouté en un excès de 10 jusqu'à 30% en poids par rapport à la composition nominale Sm₂Fe₁₇₋ₓTaₓ pour compenser des pertes par évaporation, l'addition de Ta étant comprise entre 4 et 5 at% et que cet alliage Sm-Fe-Ta est au moins refondu à trois reprises, où cette fusion est une fusion à l'arc dans une atmosphère d'Ar purifié avec Ti.
